

## UNITED STATES PATENT OFFICE

2,053,270

## PROCESSING OF TEXTILE YARNS AND MATERIALS

Camille Dreyfus, New York, N. Y., and William Whitehead, Cumberland, Md., assignors to Celanese Corporation of America, a corporation of Delaware

No Drawing. Application September 8, 1933.  
Serial No. 688,688

## 8 Claims. (Cl. 28—1)

This invention relates to the finishing and treatment of textile yarns and materials comprising organic derivatives of cellulose and the like with substances which impart thereto improved textile properties and other improved properties to which we shall refer later.

An object of the invention is the treating of a yarn comprising organic derivatives of cellulose to improve its adaptability to being formed into textiles and the ease with which it can be handled prior to weaving or knitting.

Another object of the invention is the treating of yarn comprising organic derivatives of cellulose such that various steps now necessary in the production of a textile may be dispensed with.

Other objects of the invention will be apparent from the complete specification.

In the processing of textile yarns to obtain fabricated materials of more or less suitable properties it has been necessary, prior to our present invention, to employ special winding and/or twisting operations during which the yarn was treated with special finishes or the yarn was coated with protective sizes, which operations not only involved added expense but also required the exercise of great care to prevent damage to the yarn in such processing. We have found that these difficulties may be overcome and other advantages attained by application of certain wax-like bodies to yarns, threads, etc., comprising organic derivatives of cellulose. For instance yarn coated with wax-like bodies may be wound into a solid cheese and especially in the initial winding operation. The package wound of waxed yarn is solid and non-slipping permitting the ready winding of untwisted yarns.

Many advantages lie in an ability to use yarns of no twist or of lower twist than has heretofore been possible in that such yarns are more pliable and supple and are less expensive to form. They impart more covering power and a softer handle to materials made therefrom. Further it is possible to make woven fabrics therewith with a more uniform ratio of crimpage in the warp and in the weft, thereby making firmer fabrics in which the weft slips less readily over the warp in subsequent wear. These advantages are attained in our invention by employing yarn of little or no twist, but which has been coated with wax-like bodies.

It has been the custom in the weaving of taffetas and poplin-taffetas and like fabrics to size the warp more or less heavily to protect it from chafing in the weaving process and in such quality of fabric it was necessary to weave with con-

siderable tension on the warp to avoid a defect in the fabric generally known as "frostiness". This high tension causes the warp to be comparatively straight and permits the weft to slip. By employing our invention, yarns of organic derivatives of cellulose that have been coated with wax-like bodies may be employed in the warp, which may be woven quite slackly without the appearance of any "frostiness" and with substantially more resistance to slip of the weft over the warp in subsequent wear. The organic derivative of cellulose yarn processed according to our invention permits weaving with less tension on the warp thereby forming less picks without slipping. Yarn coated with the wax-like bodies of our invention gives as high as 25% greater slipping stress than normal standard yarn.

Another difficulty that has been encountered in the processing of textile yarns of organic derivatives of cellulose is that in the circular knitting of yarns, perfect stitch shape has been extremely difficult to obtain and only then with continued and accurate machine adjustments on some yarns. This may be due largely to a varying coefficient of friction between needle, tensioning devices, guides and the yarn. With the use of organic derivative of cellulose yarn treated with wax-like bodies in accordance with our invention the tensioning devices may be eliminated and the treated yarn lubricates the guides thereby permitting perfect stitch shape. Fabrics circular knitted from organic derivative of cellulose yarn treated according to our invention do not show as many needle lines and pin holes as fabric knitted from normal yarn.

Another difficulty in the textile processing of yarns has been that in the knitting or weaving of yarns of low twist, the thread has split or divided, particularly when winding off over the head of a package, pirn, bobbin, etc., giving rise to defects in fabricated goods and a lowering of the efficiency of the process, also the thread has divided on the knitting needles in knitting processes producing what is generally known as a "needle split" and a defective place in the fabric. In accordance with our invention organic derivative of cellulose yarn of low twist and of no twist coated with wax-like bodies may be knit or woven without needle splitting or dividing of threads on the pirn, while preventing tugging tensions, drawing in of the selvedge, and otherwise imperfect fabrics.

Difficulty has always been experienced in the processing of textile materials in that oil stains contaminated with metal from bearings and the

like have been difficult to remove and for that matter dirt or contamination also. In accordance with our invention oil or other stains on fabrics may be readily scoured during normal 5 dyehouse processing to produce clean goods.

We have found that when organic derivative of cellulose yarn is treated according to our invention, it may be wound to a cheese, cone or other cross wound package at the metier, thus 10 eliminating the necessity of rewinding and twisting operations. Our invention also permits the winding of a larger cross wound package than heretofore practical. There has been a mechanical limit to the speed at which the cross wound 15 packages may be wound both in respect to damage to the yarn by very high feed rates with very high traverse speeds such as, for example, a 4" length cheese winding at 300 metres per minute with a traverse speed of 300 strokes per minute 20 and in respect to mechanical stresses resulting in damage in the traverse mechanism. Without the aid of our invention it has been impracticable to wind a cross wound package of low twist or no twist yarn as the result was a package of yarn 25 not sufficiently firm for handling and which could not be used in subsequent textile processing without slipping and entangling.

We have now found that when organic derivative of cellulose yarn is treated with wax- 30 like bodies, the traverse mechanism of a cross wound package winding device may be caused to reciprocate more slowly and/or the feed rate of the yarn may be very substantially increased without the formation of a soft or difficult package. We find that when we wind cheeses of un- 35 twisted yarn, either in the process of the initial formation of a synthetic yarn or in the textile processing of yarns, our processed yarn not only produces a solid firm package with free delivery 40 in further processing, but causes the filaments to be close together with the result that in further textile processing no matter how severe, for example warp knitting, the yarn is processed without damage or dividing of the thread. Fabrics 45 knitted of an untwisted or low twist organic derivative of cellulose yarn made possible by our invention have more covering power than those knitted from twisted yarns due to the absence of twist and the greater spread of the thread. 50 Further such fabrics have a softer and more easy handle, highly suitable, for example, in under-wear trades.

Another useful property of the organic derivative of cellulose yarns treated according to our 55 invention is that it may be wound into packages of less hardness but with adequate stability in respect to shipping in boxes and general handling, and this enables slower winds to be employed in cheeses, pincers, cones, bobbins and the like and 60 this, in turn, causes the yarn to deliver from such packages with smoother running tension in fabrication processes such as knitting, weaving, etc. on which smoother delivery there results in a more uniform fabric.

65 The process of our invention is applicable to textile yarns and like materials comprising filaments of organic derivatives of cellulose such as organic esters of cellulose and organic ethers of cellulose. Examples of organic esters of cellulose are cellulose acetate, cellulose formate, cellulose propionate and cellulose butyrate and examples of organic ethers of cellulose are ethyl cellulose, methyl cellulose and butyl cellulose. The organic derivative of cellulose filaments may 70 be substantially continuous or they may be in the

form of short lengths or staples associated together by twisting.

In accordance with our invention in any winding operation of a yarn or filament, we apply a wax-like body which is emulsifiable in water, 5 soap solution, solvents and like scouring baths. The wax-like body contains at least a proportion of one or more such emulsifiable wax-like bodies as the mono-stearate of diethylene glycol, the mono-stearate of ethylene glycol, the mono- 10 stearate of triethylene glycol, the mono- or di-stearate of glycerol, triethanolamine stearate, diethanolamine stearate, mono-ethanolamine stearate, ethylene glycol oleate, diethylene glycol oleate, triethylene glycol oleate, the mono- or 15 di-oleate of glycerol, triethanolamine oleate, diethanolamine oleate, monoethanolamine oleate or other like waxy bodies.

In place of or with the stearates and oleates 20 above specified the palmitic or other higher mono-fatty acid esters of glycol, polyglycols, glycerols and higher polyhydric alcohols may be used.

The wax-like bodies may be used alone or in 25 combination with other bodies, such as cresylic acid, butyl acetate, polymerized fatty acid and glycero or glyco boric acid or cetyl alcohol or esters or ethers of higher fatty alcohols.

Beneficial results may be obtained by incorporating 30 in the treating material mixtures of two or more of the above named compounds as will be seen from a further description of our invention.

For certain purposes it is advisable to add to any or a mixture of the above readily removable 35 wax-like bodies, a proportion of the so-called non-emulsified wax-like materials to act as sizes or hardeners such as ceresin wax, beeswax, stearic acid, stearin, palmitic acid, ozokerite wax, carnauba wax, chlorinated naphthalene and like bodies, as these when mixed with the emulsifiable 40 wax-like bodies emulsify also in water, soap solutions and the like.

For purposes of plastifying and softening these 45 wax-like bodies, we may also apply to the yarn simultaneously with the application of the wax-like body or in a separate operation, softening materials such as olive oil, oleic acid, glycols, diethylene glycol, glycerols and/or their esters and ethers. With or in place of the above plasticizers or softeners, we may apply cotton seed 50 oil, tung oil, rape seed oil and the like as carriers.

The invention is applicable to the treatment of 55 yarns or filaments, under which terms are included threads, assemblies or bundles of a number of continuous filaments which may be in parallel relationship or which may be twisted together, artificial bristles, straws, short lengths of staple fibres, or yarn spun from such staple fibres. Yarns may be employed having therein or thereupon effect material such as pigments, 60 filling materials, dyes or lakes; fire retardants such as beta chlorophthalene, triphenyl phosphate, tricresyl phosphate or the like.

The wax-like bodies may be applied in any 65 suitable manner. For example they may be applied by contacting the yarn with a wick, roller, disc or other furnishing device, feeding the wax-like body dissolved in a molten state in warm naphtha, xylene, olive oil, glycols, glycerols, triethanolamine esters and ethers or mixtures of 70 same, diethylene glycol, ethylene glycol and glycerols, mineral oil, the monomethyl or diethyl ether of ethylene glycol or their acetates, cyclohexanol, ethyl oxybutyrate, butyl alcohol, butyl acetate, ethylene diamine or other suitable solvent 75

depending on the constituents of the material forming the wax-like bodies. The solvent subsequently evaporates or dries by oxidation leaving the filaments coated with the wax-like body.

5 We may dip hanks of the yarn in such molten solution. Again we may force such molten solution through the windings of a bobbin, cheese or other package of yarn. Another modification of the process is to apply such solution by spraying.

10 If desired such wax-like bodies may be applied to the yarn in the form of aqueous emulsions by hank dipping or similar process, or the emulsion may be applied by drawing a single yarn therethrough during a winding operation. The emulsion may be applied with a roller or other furnishing device.

Alternately, the wax-like bodies may be applied to the yarn while in a molten condition, which may be conveniently accomplished by melting the wax-like bodies in a heated trough and applying the same to the yarn during a winding operation by means of a roller whose lower portion dips into the molten wax-like bodies or by any of the other furnishing means described above.

The wax-like bodies may be applied in any winding operation. For example, the wax-like body may be applied to artificial yarn immediately after they leave the spinning chambers and we have found that they are excellent lubricants for cellulose acetate yarn formed by the dry evaporative method in which process the yarn may be twisted by the cap spinning method and requires considerable lubrication to avoid chafing of the filaments on the cap edge. The wax-like bodies may also be applied in winding operations subsequent to the winding at the metier or spinning chamber, for example in unwinding a cap spun package for twisting and rewinding onto a cheese.

The suitable amount of wax-like body for application to obtain desirable textile properties will vary according to the nature of the process and the fabricated goods. The approximate amount of wax-like body applied for each particular purpose and nature of wax-like body will be apparent from the examples given. Usually we find these requirements call for an amount of a wax-like body equal to  $\frac{1}{2}$  to 20% of the weight of the yarn that is treated. The solidity of the wax and its melting point also will vary somewhat according to the wax-like bodies used, the nature of the process used and the fabric produced. Some processes call for a comparatively hard wax-like body while others call for a comparatively soft or oily wax-like body. For example, some processes appear to be improved more by the employment of a 10% finish of diethylene glycol stearate while others are improved by a finish of 5% olive oil in which has been melted 10% diethylene glycol stearate on the weight of the olive oil. By the use of hard wax-like bodies yarn may be woven as warp without any further sizing which otherwise is not the case, unsized yarn fraying and breaking in weaving.

Another modification of our process is to color the wax-like body with a fugitive color, thereby enabling identification of the thread in textile processing and enabling it to be distinguished from all other threads, which property is highly desirable, for example, where yarns of different type are employed in one construction of fabric and the pattern has to be followed by the operative in order to avoid mechanical error.

75 We find that certain of the wax-like bodies

listed above such as triethanolamine stearate or oleate have pronounced solvent power for the fugitive colors such as "Acid Green G" (Color Index No. 666), "Violet 5 BK" or "Xylene Blue" (Color Index No. 712). Likewise when we incorporate glycols or other polyhydric alcohols and/or their ethers and/or their esters, we may dissolve a tint or color in these as they are solvents for suitable fugitive colors.

By way of describing our invention still further and not with the intention of limiting its scope thereby, we give the following specific examples.

*Example I*

15 Diethylene glycol stearate which may contain some free stearic acid is taken and dissolved at 25% concentration in naphtha at 55° C. Cellulose acetate yarn is spun by the dry evaporative method at 150 denier and at 200 metres per minute 20 feed rate. The yarn is wound up and twisted to about 1 turn per inch by the cap spinning method, employing a spindle speed of around 11,000 R. P. M. In its passage from the spinning cabinet to the feed roller or anywhere else along its 25 passage between the cabinet and the bobbin, the yarn is contacted with a small steel roller rotating in the molten wax solution, rotating at a convenient speed applying 5% wax to the yarn. We find that the naphtha wax mixture remains molten and of a lubricative nature until after the yarn is wound on the bobbin and that no undesirable deposits of wax accumulate on guides, cap edges, etc.

30 This yarn may be circular knit with a multiple feed machine with spring or latch needles without further twist. Still further it may be woven in warp without further twist or without sizing of the yarn and at substantially lower warp tensions, thereby avoiding much accidental strain of 35 warps with the production of streakiness and improving the solidity of the fabric in respect to slip of weft over warp. For example, in a fabric of the following construction, we have found an improvement of 50% in the resistance of slip of 40 the weft over the warp when compared with a 45 similar fabric produced by the normal methods involving sizing of the warp.

|                                           |    |    |
|-------------------------------------------|----|----|
| Warp—Cellulose acetate yarn—150 denier    | 40 | 50 |
| filaments 0.9-1 turns per inch.           |    |    |
| Weaving reed—42 dents per inch            |    |    |
| Reed width—40 $\frac{3}{4}$ "             |    |    |
| Width through reed with edges—39.69"      |    |    |
| Number of ends per dent—2                 |    |    |
| Total ends in warp without edges—         | 55 |    |
| 3334                                      |    |    |
| Nature of entering and number of          |    |    |
| shafts—6 skip                             |    |    |
| Weave—tabby                               |    |    |
| Filling—Cellulose acetate yarn—150 denier | 40 | 60 |
| filaments 0.9-1 turns per inch            |    |    |
| 60 picks per inch                         |    |    |
| Raw width—39 $\frac{1}{2}$ "              |    |    |
| Dyed and finished width—39"               |    | 65 |

We find also that by twisting the warp of the waxed yarn  $2\frac{1}{2}$  turns per inch, this increased resistance to slip is not reduced.

In respect to the circular knit fabric, this knits with a perfect stitch shape and without rowiness, 70 even when the twist of the yarn is reduced to 0.9 turns per inch.

Still further, we find that such yarn may be pirned and woven as weft, for example, in the same construction as we have above specified. 75

Without the wax on the yarn, the thread splits and the filaments chafe on the purn tube also the thread divides around the tube causing fabric defects. With the wax-like bodies, however, 5 present on the yarn, the filaments adequately lie together. Fabrics produced with this 1 turn per inch in the weft and warp have more cover and are substantially softer than those heretofore produced which have had at least 2.5 turns per 10 inch in both weft and warp.

#### Example II

We repeat Example I using triethanolamine stearate or diethanolamine stearate or mono-15 ethanolamine stearate, instead of the diethylene glycol stearate.

#### Example III

We repeat Example I employing any mixture 20 of diglycol stearate and triethanolamine stearate.

#### Example IV

We repeat Examples I, II and III employing partly or wholly palmitic acid as the fatty acid 25 radical in place of stearic acid.

#### Example V

We repeat Example I substituting a mixture of 30 parts triethanolamine stearate and 20 parts 30 ozokerite wax.

#### Example VI

During the winding and twisting of 75 denier cellulose acetate yarn to 28 turns per inch for 35 subsequent weaving as warp and weft in a voile or ninon type of fabric, we contact the yarn with a furnishing roller rotating at suitable speed in a trough containing molten diethylene glycol stearate or any wax mixture in the preceding 40 examples thereby imparting to the yarn 2-3% of such wax. In subsequent weaving of the fabric, we find that we may weave with slacker tensions thereby avoiding strain and at the same time find that we may weave with much more 45 uniformity of appearance and straightness of pick than we can without the presence of such wax on the yarns which is normally woven without any size.

#### Example VII

50 We repeat Example I but instead of dissolving the diethylene glycol stearate in warm naphtha, we apply to the yarn a molten mixture of 50 parts by weight of olive oil and 50 parts by weight 55 of diethylene glycol stearate. This imparts a softer waxing to the yarn and is more suitable for closely knitted warp knit or circular knit goods than for weaving.

#### Example VIII

60 We repeat Example VII employing 95 parts diethylene glycol stearate and 5 parts olive oil and dissolve these at 30% concentration in warm naphtha. This finish is more suitable for closely 65 woven goods.

#### Example IX

We prepare a molten mixture of diethylene 70 glycol 50 parts, triethanolamine stearate 50 parts and xylene blue 2 parts and apply this as in Example I molten at approximately 55° C. This is an excellent knitting finish and the yarn is tinted a distinctive green-blue. The yarn scours readily in warm water and the color is fugitive to all 75 yarns in neutral and alkaline baths.

#### Example X

We prepare a molten mixture of 75 parts naphtha, 23 parts triethanolamine stearate and 2 parts violet 5 BK and apply this as in Example I at 55° C. This is also an excellent knitting or weaving finish suitable for both weft and warp in woven goods and scours readily in warm water and does not color any other yarns in neutral or alkaline baths.

10

#### Example XI

An emulsion is prepared of 1.5% diethylene glycol stearate and 98.5% water at 65° C. Hanks of cellulose acetate yarn are immersed and worked in this and then allowed to air dry after which they are rewound on a suitable package. This applies approximately 3% of the emulsifiable wax to the yarn and the improved textile properties of preceding examples are imparted to the 20 yarn.

#### Example XII

Example XI is repeated, employing mono-25 ethanolamine stearate instead of diethylene glycol stearate.

While in the foregoing specification we have cited specific instances and examples, as we have stated it is not our intention to limit the scope of our invention thereby. Obviously many modifications may be employed without departing from the spirit of the invention.

Emulsifiable waxes and their adulterants, tints, hardeners and softeners may be applied in any textile processing either molten or from solution such as in twisting, purning, warping, slasher sizing. Goods made from such yarns may be treated by any scouring and dyeing process, for instance, on winches, jigs, open soapers, in hanks of fabric, on the string and so on. The waxes emulsify readily and have the peculiar advantage of remaining in a finely divided state of emulsion even after cooling, thereby passing through drain lines, etc. without any choking.

All fabrics made according to the process of our invention, in scouring, shed dirt marks, oil 45 stains and the like, remarkably freely and quickly as we have before stated. An obvious modification of our process is to scour such goods only partially, which partial scouring may be effected by scouring at a temperature barely at the melting point or temperature required to emulsify the wax or giving a short restricted scour, for instance, on the jig, thereby removing only part of the wax and imparting to the yarn a less soft handle which is frequently desired for trimming effects in millinery and like trades. The obtaining of such stiffer properties may also be controlled by including in the wax more of a non-emulsifiable body such as ozokerite wax, paraffin wax and like substances.

In the above examples glycol ethers and/or their esters may be employed as addition and carrying agents. Also to any of the above wax-like bodies triethanolamine may be added to dissolve free stearates etc. or ethylene-diamine may be used in place of or with the triethanolamine.

Sulphonated naphthalene may be added to the mixture such as diethylene glycol stearate and mineral oil. When a wax-like body is carried in a light mineral oil and applied to the yarn while 70 molten or in solution it forms a transparent covering making possible the selection of lustre.

Stockings knitted from yarn processed with the wax-like bodies may be dyed in a nest in a "drum" machine without prominent creases, and 75

without the necessity of delustering them by boiling beforehand.

The yarn processed with the wax-like bodies meets the demand for a good soft size in the 5 ribbon trade.

The application of the wax-like bodies to a yarn reduces considerably the amount of static electricity generated in the future processing of the yarn thereby preventing separation of the 10 filaments with resulting better cover properties and less breaks. The property of the yarn to generate static charges is especially reduced if there is a slight excess of triethanolamine, ethylene-diamine or similar compounds present 15 in the wax-like solution.

Wax-like bodies with or without softeners, carriers, addition agents, sizes, dyes, or effect materials may be applied to staple fibres made 20 of cellulose acetate or other organic derivative 20 of cellulose either prior to their being cut from continuous filaments, or after their formation, or after spinning thereby preventing "ball" effects on the fabric made therefrom. The balling effect is caused by the loose ends rubbing into a 25 knot over the surface of a knit fabric.

By way of describing our invention still further and not with the intention of limiting its scope thereby, we give the following specific examples of winding our treated yarn.

#### 30 Example XIII

We spin at a feed rate of 120 metres per minute by the dry evaporative method an acetone soluble cellulose acetate yarn of 150 denier 40 filaments 35 with little or no twist and wind directly onto a cheese. Between the thread exit guide from the spinning cabinet and the cheese we cause the 40 yarn to contact with a furnishing roller or other suitable device furnishing 4% diethylene glycol 45 stearate from a 30% solution in naphtha at 50° C. The traverse speed of 125 strokes per minute is maintained. The cheeses wound on tubes of 1½" diameter and 4" in length and up to 4½" in diameter, thus making cheeses containing 50 ing two or more pounds of yarn. The cheeses so obtained are firm and may be shipped even with vigorous handling without becoming softened or losing their ability to deliver freely and cleanly in subsequent textile processing and exhibit other improved properties.

#### Example XIV

We repeat Example XIII, that is the winding of cellulose acetate yarn in the process of its 55 formation onto cheeses with a traverse average speed of 125 strokes per minute but increase the feed rate of the yarn to 300 metres per minute. The cheeses so formed have substantially the same desirable properties as those similarly 60 wound but wound at 240 metres per minute.

#### Example XV

We repeat Example XIV with a feed rate of 200 metres per minute and reduce the amounts 65 of wax-like body to 2% with substantially the same results.

The treating of yarn with wax-like bodies enables the use and handling of untwisted or low twist yarn for purposes and in like manner to 70 the twisted yarn. The covering of synthetic yarn at the metier with a wax-like body gives better ageing qualities to the yarn. The wax-like bodies retard the evaporation of the cellulose solvent, as acetone, keeping the yarn in better 75 knitting condition.

In the foregoing specification we have cited specific instances and examples, but it is not our intention that the scope of our invention should be limited thereby, as obviously many modifications may be made without departing from the spirit of the invention. Obviously such 5 yarn may be treated with the wax-like bodies before, between, after or during twisting operations or winding operations. The wax-like bodies may be incorporated in the spinning dope or 10 inserted into the yarn by the action of swelling agents.

Having described our invention, what we desire to secure by Letters Patent is:

1. Method of improving the textile properties of 15 yarns or filaments containing substitution derivatives of cellulose in which the substituent group is organic, which comprises forming a coating thereon by applying thereto a molten wax-like body, selected from the group consisting of the 20 higher fatty acid esters of di- and poly-hydric alcohols and the salts of alkyloamines with higher fatty acids, in the absence of water, said wax-like body being inherently readily removable by scouring with aqueous liquid, and thereafter causing 25 the wax-like body to solidify on said yarns or filaments by cooling.

2. Method of improving the textile properties of 30 yarns or filaments containing cellulose acetate, which comprises forming a coating thereon by 30 applying thereto a molten wax-like body, selected from the group consisting of the higher fatty acid esters of di- and poly-hydric alcohols and the salts of alkyloamines with higher fatty acids, in the absence of water, said wax-like body being 35 inherently readily removable by scouring with aqueous liquid, and thereafter causing the wax-like body to solidify on said yarns or filaments by cooling.

3. Method of producing fabric of improved 40 properties, which comprises applying to yarn, containing cellulose acetate and not having a twist of more than 1.5 turns per inch, a molten wax-like body, selected from the group consisting of the higher fatty acid esters of di- and poly- 45 hydric alcohols and the salts of alkyloamines with higher fatty acids, in the absence of water, said wax-like body being inherently readily removable by scouring with aqueous liquid, causing the wax-like body to solidify on said yarn by cooling, forming said wax-coated yarn into fabric and 50 then scouring said fabric with aqueous liquid.

4. In the method of producing a spun yarn comprising staple or short lengths of filaments 55 containing a substitution derivative of cellulose in which the substituent group is organic, the step of applying thereto a molten wax-like body, selected from the group consisting of the higher fatty acid esters of di- and poly-hydric alcohols and the salts of alkyloamines with higher fatty 60 acids, in the absence of water, said wax-like body being inherently readily removable by scouring with aqueous liquid, and causing said wax-like body to solidify on said filaments by cooling.

5. A solid, non-slipping, cross-wound package 65 of the flangeless type comprising yarns containing a substitution derivative of cellulose in which the substituent group is organic, said yarns not having a twist of more than 1.5 turns per inch and being coated, in the absence of water, with a wax- 70 like body, selected from the group consisting of the higher fatty acid esters of di- and poly-hydric alcohols and the salts of alkyloamines with higher fatty acids, said wax-like body being inherent- 75

ly readily removable by scouring with aqueous liquid.

6. A solid, non-slipping, cross-wound package of the flangeless type comprising yarns containing cellulose acetate, said yarns not having a twist of more than 1.5 turns per inch and being coated, in the absence of water, with a wax-like body, selected from the group consisting of the higher fatty acid esters of di- and poly-hydric alcohols and the salts of alkyolamines with higher fatty acids, said wax-like body being inherently readily removable by scouring with aqueous liquid.

7. A fabric comprising yarns containing cellulose acetate and not having a twist of more than 1.5 turns per inch and coated, in the absence of

water, with a wax-like body, selected from the group consisting of the higher fatty acid esters of di- and poly-hydric alcohols and the salts of alkyolamines with higher fatty acids, said wax-like body being inherently readily removable by scouring with aqueous liquid.

8. A knit fabric comprising yarns containing a substitution derivative of cellulose in which the substituent group is organic, said yarns not having a twist of more than 1.5 turns per inch and being coated, in the absence of water with diethylene glycol stearate, said diethylene glycol stearate being inherently readily removable by scouring with aqueous liquid.

CAMILLE DREYFUS.

WILLIAM WHITEHEAD.

15